

1,000,330.

N. DODGE.  
SECONDARY OR STORAGE BATTERY.  
APPLICATION FILED JUNE 9, 1904.

Patented Aug. 8, 1911.



Fig. 1



Fig. 2

Oppressor  
Frank E. French

Inventor  
Norman Dodge  
Aug. 8, 1911  
Augustine D. Stoughton  
Attorneys

# UNITED STATES PATENT OFFICE.

NORMAN DODGE, OF PHILADELPHIA, PENNSYLVANIA, ASSIGNEE TO THE ELECTRIC STORAGE BATTERY COMPANY, OF PHILADELPHIA, PENNSYLVANIA, A CORPORATION OF NEW JERSEY.

## SECONDARY OR STORAGE BATTERY.

1,000,330.

Specification of Letters Patent.

Patented Aug. 8, 1911.

Application filed June 9, 1904. Serial No. 211,739.

*To all whom it may concern:*

Be it known that I, NORMAN DODGE, a citizen of the United States, residing at the city of Philadelphia, in the county of Philadelphia and State of Pennsylvania, have invented certain new and useful Improvements in Secondary or Storage Batteries, of which the following is a specification.

10 The object of the present invention is to provide a satisfactory and efficient wood separator and to provide for treating the same in such a way as to make it practically successful in its application to lead storage batteries.

15 To this and other ends hereinafter set forth, the invention, stated in general terms, comprises the improvements to be presently described and finally claimed.

20 The nature, characteristic features and scope of my invention will be more fully understood from the following description taken in connection with the accompanying drawings forming part hereof and in 25 which—

Figure 1, is an elevational view and Fig. 2, is a sectional view of a storage battery embodying features of the invention.

25 In the drawings *a*, is a storage battery separator consisting of wood adapted to constitute a diaphragm impervious to battery sediment. Bass, birch, cherry, white pine, poplar and Oregon pine are types of such wood. The shape of the separator *a*, shown in the drawings is merely selected for illustration and the type and arrangement of the plates *b* and *c*, are likewise illustrative only. These details form no part of the invention.

30 The wood separator which is adapted to constitute a diaphragm impervious to battery sediment is primarily deprived of such of its constituents and wood acids as would in the operation of a battery attack lead.

35 Acetic acid is a type of the wood acids referred to and if the latter were present they would in the operation of the battery either attack the positive lead pole plate causing its disintegration or perhaps by 40 oxidation escape without doing injury, but

the only successful course is to primarily deprive the wood of such acids. There are two ways of treating the wood for the accomplishment of this result. First, the wood is soaked in a sulphuric acid water 55 solution, of, for example, 1.2 specific gravity at normal temperature for two days, more or less. If the solution is heated, for example to 100 degrees F. weaker acid can be used, for example, 1.1 specific gravity, 60 the duration of the treatment being about the same, and second; the wood is soaked in an alkaline solution such as a 3% solution of caustic potash at normal temperature for about 24 hours. Subsequently the 65 wood is washed as in running water for 48 hours, more or less. One pound of the dry alkali is sufficient for treating five pounds of dry wood. The use of heat operates as an accelerant with both the acid and alkaline solutions. The effect of the treatment with mild acid solution or with mild alkaline solution is to remove from the wood those acids or constituents which in the use 70 of the battery are likely to attack and disintegrate the lead of the positive pole plate. Although the wood is by the described treatment deprived of certain of its constituents, still it retains others of its constituents, some or all of which beneficially 75 affect the operation of the battery, more particularly in respect to the capacity and life of the negative pole plates. The treated wooden separators are characterized by the property of warping, shrinking, curling and splitting when dry so that they are kept 80 wet or impregnated with moisture until they are placed in the battery liquid.

85 It will be obvious to those skilled in the art to which my invention relates that modifications may be made in details without departing from the spirit thereof, hence the invention is not limited otherwise than as the prior state of the art may require, but

90 Having thus described the nature and objects of my invention, what I claim as new and desire to secure by Letters Patent is:

95 A storage battery separator consisting of a sheet of fine grain wood having its natural structure and containing its cellulose and 100

fibrous constituents and constituting a dia-  
phragm impervious to battery sediment and  
primarily deprived of such of its constitu-  
ents as would deleteriously attack lead  
5 when subjected to electrolytic action and  
retaining such of its constituents as bene-  
ficially affect a negative pole plate.

In testimony whereof I have hereunto  
signed my name.

NORMAN DODGE.

Witnesses:

W. J. JACKSON,  
FRANK E. FRENCH.